

## UNITED STATES PATENT OFFICE

2,178,770

PULVERULENT DRY COMPOUND FOR FORM-  
ING PAINTS, PLASTICS, AND CEMENTSWilliam Zaisser, Woodside, N. Y., assignor of  
one-half to Harry S. Walker, New York, N. Y.No Drawing. Application April 6, 1938,  
Serial No. 200,426

31 Claims. (Cl. 106—32)

The present invention relates to an improvement in a compound, useful for making paint, or for making plastic cementing compounds. In some of its forms, it may also be useful in road 5 surface making.

One of the important, underlying features of the present improvement lies in the provision of a base, or vehicle for the various aggregates that have been found useful, for wide varieties of application in this art, as will hereinafter be noted in detail.

The base above noted comprises a pulverulent, dry, asphalt, bitumen or mineral pitch, into which is intimately mixed dry, pulverulent aggregates or materials, either in single or compounded combinations, depending upon the use to which the compound may be put.

The volumetric proportions of the different, dry aggregates are varied, depending on the type of use, as desired, such variations being well within, and without destroying, the bonding power of the base.

Another important feature is that the mixed compound, may, after dry mixing, be dispensed in its dry form in containers, for mixing with a liquid base solvent, or fluid by the user, as desired, thereby to liquefy the base, to act as a bond; and as thus dry dispensed, detrimental reaction is eliminated, the aggregates or materials having in their dry, pulverulent, comminuted, or shredded state, no detrimental reaction with the dry, pulverulent mineral pitch base.

One of the principal features of the herein improvement, is in the use of the dry powdered or comminuted aggregates, whereby to color, alter the nature of, or otherwise utilize the base as a vehicular bond, the use of said dry, varient and intermixed aggregates positively preventing the coalescing of the powdered mineral pitch or tar. Thus the natural tendency of the powdered base when stored in containers, alone, to fuse into a solid body, is eliminated, the powdered mix being thus shippable and storable in its dry form until used. The prevention of coalescence of the dry mix retains it in open, substantially porous condition, whereby, when the user receives the contained dry mix, he may mix into it a suitable solvent, to reduce the aggregates to such desired consistency, or plasticity, as the use requires.

While any form of the present compound may be standard as to stated uses, its viscosity, when mixed with different volumes of solvent, may vary from a thick, heavy non-flowing cement, to a free flowing liquid condition, whereby it may be 55 brushed on, like paint.

Where the compound is heavy and non-flowing it may be used as a weatherproofing crack filler, or on roofing and the like. When the compound is mixed with a greater amount of solvent, it may be brush-applied as a protective surface 5 coating.

The aggregates that may be mixed with the pulverulent base, in addition to preventing the powdered base from coalescence, may provide for different colored compounds, may also provide 10 for different degrees of hardness, and may be adapted for a wide variety of physical embodiments, without violating the one underlying principle of the use of a pulverulent pitch of coalescing nature, wherein the intermixing therein 15 of the dry, pulverulent non-analogous material performs two functions, one, to prevent the natural coalescence of the pitch, the other to provide a color, or equivalent useful ingredients therein.

The use of some of the hereinafter noted aggregates, in addition to the foregoing noted physical functions also reduce the cost of the present compound, inasmuch as some of said aggregates are extremely low in price and are customarily sold in bulk form. Thus the aggregate forming 20 materials in many instances act also as fillers in 25 addition to the other functions.

A list of the preferred forms of aggregates is given below, and while it shows the preferred materials, it does not exhaust the possibilities of 30 use of other aggregate forming materials, not listed herein.

The preferred aggregate-forming, filler materials in dry pulverulent or ground condition are as follows:

## List #1

|                     |                  |
|---------------------|------------------|
| Alabaster           | Magnesite        |
| Asbestos            | Marble dust      |
| Alberine stone      | Plaster of Paris |
| Cardboard           | Portland cement  |
| Cala stone          | Paper            |
| Cork                | Stone            |
| Cellulose           | Sawdust          |
| Diatomaceous earth  | Slate flour      |
| Felt                | Steatite         |
| Ground rubber scrap | Sand             |
| Graphite            | Silica sand      |
| Hydrated lime       | Sea sand         |
| Kaolin              | Talc             |
| Lime stone          | Wood flour       |
| Leather             |                  |

These various aggregates, or materials, may be powdered or shredded, according to their natures and desired functions.

For coloring the base, dry, pulverulent colors are used, these being mixed with the base in the same manner as indicated for the filler aggregates, and the dry colors, alone, with the base, perform the double function of preventing coalescing of the powdered bitumen or tar, in addition to color blending the same.

A preferred list of dry, pulverulent bitumen coloring material is listed below, and it is to be understood that this list is incomplete, and not limiting in any sense, because of the obviously greater number of variations of colored materials that may be used, and are available.

Many of the powdered metal oxides are useful in the present improvement, such as

*List #2*

|                                                                  |            |
|------------------------------------------------------------------|------------|
| Cuprous oxide                                                    | White lead |
| Lime oxide.                                                      | Zinc oxide |
| 20 Mercuric oxide                                                |            |
| also some of the colored and powdered earths are useful, such as |            |

*List #3*

|                |              |
|----------------|--------------|
| 25 Burnt umber | Sienna       |
| Fuller's earth | Yellow ochre |

Other filler and coloring aggregates are useful, when mixed in the base, for toxic insecticidal and bacteriacidal purposes, these aggregates performing the triple function of preventing coalescence of the base, coloring the same and preventing insect and bacterial attacks upon the objects coated with such toxic aggregates, these being noted, below, as follows:

*List #4*

|                   |             |
|-------------------|-------------|
| Cuprous oxide     | Paris green |
| Electric bronze   | Red lead    |
| 40 Mercuric oxide |             |

The foregoing toxic aggregates are waterproof and are particularly useful for protecting boat hulls, piling and woodwork from attacks by barnacles, teredo worms, termites and ants.

From the foregoing disclosure, it is obvious that any single filler, color, or toxic aggregate may be selected and mixed with the bitumen base, or any predetermined combination of aggregates from each of the four lists above outlined, may be used, to suit varying known conditions. Such combinations may be prescribed, for utilizing the desired functional features of each aggregate. Further, such combinations, organic, and mineral, excepting hydrated, powdered lime, have no reaction with each other when dry mixed with the powdered dry bitumen or tar, nor have they any reaction with the dry pulverulent base. Where hydrated lime is used as a hardener, with color it is necessary to select a lime proof color.

In some forms of the compound there may be required besides the powdered pitch base, a color blending, filler aggregate, such as a metal oxide, which may be red oxide, in sufficient volume to give the desired tone of red shade. Red oxide is inert and non-absorbent. A further filler aggregate desired may be of an absorbent nature such as ground wood, sawdust, or ground felt. After the intermixing of these selected aggregates and base, there remains a flowable dry compound, which when packed, remains in this condition for an unlimited period, ready for use, by the introduction of a solvent.

The user may furnish his own liquid base solvent, in desired quantities, to make a plastic

cement, or a fluid brushable coating. Such solvents may be turpentine, kerosene, gasoline, naphtha, benzine, and similar volatile fluids, and the amount of solvent used determines whether the final dissolved compound is used as a brush coating, paint or a plastic, light or heavy, for cementing or puttying. Thus the user determines the degree of viscosity of the final compound, in accord with the use to which the final compound is put.

In some forms of use, the dry compound may comprise a mixture of bronze powder, powdered bitumen and hydrated lime, in proportions of one part bronze powder (of any color) one part bitumen powder and one part hydrated lime. The lime is included to act as a hardener, after the compound is applied.

The specific proportions above given may be varied, to meet encountered conditions, and the proportionate volumes of the base to the volume of the dry mix may vary from one part each, of each aggregate, to one part powdered bitumen or pitch, to as high as fifty parts of each of the three elements of the compound. There is no hard and fast rule as to the proportions used because of the requirements of different colors, or tonal shades of each color desired, and the different functions and uses to be met.

It has been found that the introduction into the mix of talc gives the final compound, when used as a paint, the property of smooth flowability and easy brush action. Talc, or graphite, thus used, may be of any proportional volume to the volume of the powdered pitch used, as the use of talc or graphite changes the color of the final paint, and the volume of talc or graphite thus used, may be varied, for color purposes up to the bonding power of the base.

Such volumes of talc or graphite and pitch may be varied from one part talc or graphite to sixteen parts of powdered pitch, or to fifty parts of each ingredient, depending on the color desired. More talc or graphite makes the final paint extremely smooth to apply, causes the final paint, when dry to have a distinct sheen or gloss, which may be heightened by polishing or rubbing.

Talc is also included in the mix, where colors are used, such as colored bronze powders, dry pulverulent colors, metal oxides to lighten the colors from their base shade to the desired lighter tones.

Where hydrated lime is used as an aggregate for hardening with a color, it is necessary to pack the dry mix in an air tight container, to prevent atmospheric action on the lime, with a consequent degradation of the contained color.

In mixes where color and hydrated lime is used with the powdered pitch or bitumen, the proportions of the aggregates may be twenty five to fifty parts of powdered pitch by volume, to fifty to seventy five parts by volume of an aggregate, of which twenty five to fifty percent of lime is included, the remainder of the aggregate constituting twenty five to fifty percent of coloring matter, including bronze powder.

The proportions, wherein a filler and color is used, may also be utilized, wherein the pulverulent base of powdered mineral pitch may be used, from twenty five and fifty parts, by volume, and fifty to seventy parts, by volume, of an aggregate filler, said filler, such as shredded asbestos, constituting twenty five to fifty percent of shredded asbestos, about twenty five percent of

hydrate of lime and twenty five to fifty percent of bronze powder.

In some forms, for paint, the volume of talc and dry pulverulent pitch may be twenty percent talc to eighty percent pitch, which when mixed with a solvent of sufficient volume produces a protective brush coating of smooth nature and of a good gloss.

Good color combinations, including bronze powders, where a coloring aggregate is used, are obtained by a combination of powdered pitch, color and talc, in one third parts of each, intermixed. Variations of the proportions of ingredients noted may be used up to the bonding power of the base pitch, thereby to obtain changes in color.

An elastic, mastic crack filler is obtained by a mixture of ground rubber scrap and powdered pitch which may also include proportions of sand, ground leather scrap, ground felt, ground paper, ground cork, which enhance the elasticity of the mastic thus created and prevent the dry mix from coalescing, during storage.

Plastic mixtures of powdered pitch and Portland cement, and in some instances, a proportion of sand, form a satisfactory waterproof cement mortar, which may be trowelled on the surfaces to be protected, when admixed with a suitable proportion of solvent.

In road surfacing coatings, a mixture of sand and pulverulent pitch, dissolved in a suitable proportion of solvent, provides a good tractive surface. Other inexpensive aggregates or fillers may also be used for this purpose.

The proportions of aggregates of varying nature, either single, or in combination, may be used, as will be noted from the foregoing disclosure. The viscosities, from paints to mastics, or heavy plastic compounds, may be varied to suit the desired or indicated uses, this being accomplished by the use of properly proportioned solvents, more or less, as the type of material requires.

From the foregoing, it will be noted that the proportions and kinds of aggregates may be varied from one part aggregate to ninety nine parts of pulverulent pitch, and up to sufficient parts of aggregates up to the bonding power of the pulverulent pitch.

It is also obvious that the coating may be varied in color, nature and viscosity, as required, by the utilization of powdered, shredded or granular aggregates of different natures and functions, as mixed with the powdered pitch, for the purposes mentioned.

It is also to be noted that modifications may be made in the mixes herein noted, without departing from the spirit hereof or the scope of the appended claims.

This application is a continuation in part of my copending U. S. application No. 688,033 filed Sept. 2, 1933, for Dry compound for forming paints, plastics and cements.

Having thus described the invention what is claimed is:

1. A dry, coating compound comprising a dry pulverulent pitch, having a tendency to coalesce in storage, and a dry pulverulent aggregate admixed therewith, to prevent coalescence of the mix; the pitch being finely pulverized enough to be quickly and completely dissolved by a suitable cold solvent to form a freely flowing easily brushable paint.

2. A dry, coating compound comprising a dry pulverulent pitch, having a tendency to coalesce

in storage, and a dry pulverulent aggregate intimately admixed therewith, said aggregate constituting a mixture of a filler and a pulverulent color blending aggregate, said aggregate preventing the coalescence of the pitch; the pitch being finely pulverized enough to be quickly and completely dissolved by a suitable cold solvent to form a freely flowing easily brushable paint.

3. A dry, coating compound comprising a dry pulverulent pitch, having a tendency to coalesce in storage, and a dry pulverulent aggregate intimately admixed therewith, said aggregate coating the particles of the pitch to separate said particles to prevent coalescence thereof, during storage; the pitch being finely pulverized enough to be quickly and completely dissolved by a suitable cold solvent to form a freely flowing easily brushable paint.

4. A dry, coating compound comprising a dry pulverulent pitch, and a dry aggregate intimately admixed therewith, said aggregate maintaining the admixed compound porous and preventing coalescence of the compound during storage; the pitch being finely pulverized enough to be quickly and completely dissolved by a suitable cold solvent to form a freely flowing easily brushable paint.

5. A coating compound comprising a dry, powdered mineral pitch, the particles of which are segregated by a non-interacting pulverulent filler, to prevent coalescence of the pitch during storage; the pitch being finely pulverized enough to be quickly and completely dissolved by a suitable cold solvent to form a freely flowing easily brushable paint.

6. A plastic forming elastic, crack filling compound, comprising a dry, pulverulent pitch and an aggregate comprising, in part, a ground rubber scrap.

7. A paint forming compound, comprising a dry, pulverulent mineral pitch and a dry, color blending aggregate intimately admixed therewith; the pitch being finely pulverized enough to be quickly and completely dissolved by a suitable cold solvent to form a freely flowing easily brushable paint.

8. An insecticidal and bactericidal coating compound, comprising a dry, pulverulent mineral pitch and a dry, powdered aggregate intimately admixed therewith, said aggregate comprising a toxic material.

9. A compound adapted to be admixed with a liquid to provide a coating containing 25 to 50 parts by volume of powdered mineral pitch; and 50 to 75 parts by volume of an aggregate containing 25 percent to 50 percent hydrate of lime, and 25 percent to 50 percent bronze powder, substantially as described; the pitch being finely pulverized enough to be quickly and completely dissolved by a suitable cold solvent to form a freely flowing easily brushable paint.

10. A compound adapted to be admixed with turpentine or the like whereby to provide a preservative coating, said compound containing 25 to 50 parts by volume of powdered mineral pitch; and 50 to 70 parts by volume of an aggregate mixed with the pitch and containing 25 percent to 50 percent shredded asbestos, said aggregate containing also about 25 percent hydrate of lime, and 25 percent to 50 percent of bronze powder; the pitch being finely pulverized enough to be quickly and completely dissolved by a suitable cold solvent to form a freely flowing easily brushable paint.

11. An article of manufacture adapted for

shipment, storage and sale, comprising an air-tight container; and a composition of dry powdered material sealed air-tight therein and adapted to be admixed with an evaporable solvent to provide a flowable mass, said composition comprising 25 to 50 parts by volume of finely powdered mineral pitch; and an aggregate intimately mixed with the pitch.

12. An article of manufacture adapted for shipment, storage and sale, comprising an air-tight can; and a composition of dry powdered material sealed air-tight therein and adapted to be admixed with turpentine or the like to provide a flowable mass adapted to be applied as a preservative coating adapted to harden, said composition comprising 25 to 50 parts by volume of finely powdered mineral pitch; and 50 to 75 parts of a dry powdered aggregate intimately mixed with the pitch; said pitch and aggregate, when dry being free of affinity for, or interreaction with, each other; said aggregate being adapted to serve the multiple function of retaining the pitch evenly distributed throughout the composition and mechanically separating the particles of pitch during shipment to prevent the compacting of the pitch particles together during storage and shipment, and to retain the pitch particles separated for the easy access of the solvent thereto, and to give body to the flowable mass, and body and appearance to the final hardened product.

13. An article of manufacture adapted for shipment, storage and sale, comprising an air-tight can; and a composition of dry powdered material sealed air-tight therein and adapted to be admixed with turpentine or the like to provide a flowable mass adapted to be applied as a preservative coating, said composition comprising 25 to 50 parts by volume of finely powdered mineral pitch; and 50 to 75 parts of an aggregate intimately mixed with the pitch and containing shredded asbestos, hydrate of lime and bronze powder; said pitch and aggregate, being dry, being free of interreaction; said aggregate serving the multiple function of retaining the pitch evenly distributed and mechanically separating the particles of pitch during shipment to prevent the compacting of the pitch particles together during storage and shipment, and to retain the pitch particles separated for easy access of the solvent thereto, and to give body to the flowable mass, and body and color to the final hardened product.

14. A composition adapted to be mixed with a liquid to provide a mass suitable for filling cracks and making expansion joints, said composition comprising a binder material; and divided elastic filler material mixed with the binder material.

15. A composition adapted to be mixed with a liquid to provide a flowable mass, said composition comprising finely divided binder material tending to cake when unmixed; and divided filler material mixed with the pitch, the quantity of binder material being sufficient to form a binder and continuous cover for the flowable mass; the quantity of filler material being sufficient to prevent the binder material from caking; the pitch being finely pulverized enough to be quickly and completely dissolved by a suitable cold solvent to form a freely flowing easily brushable paint.

16. A composition adapted to be mixed with a liquid to provide a flowable mass or paint, said composition comprising finely divided pitch; and divided filler material mixed with the pitch; the

quantity of pitch being sufficient to form a binder and continuous pitch cover for the flowable mass; the quantity of filler material being sufficient to prevent the pitch of the mixture from caking; the pitch being finely pulverized enough to be quickly and completely dissolved by a suitable cold solvent to form a freely flowing easily brushable paint.

17. A composition adapted to be mixed with a liquid to provide a flowable mass; said composition comprising 25 to 50 parts by volume of finely divided pitch; and divided filler material mixed with the pitch; the pitch being finely pulverized enough to be quickly and completely dissolved by a suitable cold solvent to form a freely flowing easily brushable paint.

18. A composition of dry powdered material adapted to be mixed with a liquid to provide a flowable mass or paint, said composition comprising 25 to 50 parts by volume of finely divided pitch; and divided filler material mixed with the pitch; the quantity of pitch being sufficient to form a binder and continuous pitch cover for the flowable mass; the quantity of filler material being sufficient to prevent the pitch from caking before mixing with the liquid; the pitch being finely pulverized enough to be quickly and completely dissolved by a suitable cold solvent to form a freely flowing easily brushable paint.

19. A composition adapted to be mixed with a liquid to provide a flowable mass or paint, said composition comprising finely divided binder material; and divided slippery filler material intimately mixed with the binder material; the quantity of binder material being sufficient to form a binder and continuous cover for the filler material; the smoothness and quantity of filler material being sufficient to give to the mass gloss and smooth flowability.

20. A composition adapted to be mixed with a liquid to provide a mass or paint, said composition comprising a pitch; and finely divided talc; the pitch being finely pulverized enough to be quickly and completely dissolved by a suitable cold solvent to form a freely flowing easily brushable paint.

21. A flowable mass or paint comprising a mixture of pitch, a liquid and finely divided talc, the quantity of pitch being sufficient to form a binder and continuous cover for the talc; the talc being adapted to give to the mass or paint a gloss or sheen; the pitch being finely pulverized enough to be quickly and completely dissolved by a suitable cold solvent to form a freely flowing easily brushable paint.

22. A flowable mass or paint, comprising finely divided talc intimately mixed with a solution of pitch, the quantity of pitch being sufficient to form a binder and continuous cover for the talc; the quantity of talc being sufficient to give to the mass or paint a smooth flowability and a gloss or sheen which may be heightened by polishing.

23. A composition of dry powdered material adapted to be mixed with a solvent to provide a flowable mass or paint, said composition comprising finely divided pitch; and finely divided talc intimately mixed with the pitch; the quantity of pitch being sufficient to form a binder and continuous cover for the talc, and a continuous pitch cover for the flowable mass and the structure to which it is applied; the quantity of talc being sufficient to prevent the pitch from caking during storage and shipping, and to give to the mass

or paint a smooth flowability and a gloss or sheen which may be heightened by polishing.

24. A method for making paint, said method comprising intimately mixing pulverized pitch and pulverized slippery material; and adding a sufficient quantity of a suitable solvent for the pitch to completely dissolve the pitch; the proportion of solvent material and material being such that the pitch forms a binder and continuous cover for said material, and a continuous pitch cover for the flowable paint and the structure to which it is applied; the slippery material giving to the paint a smooth flowability and a gloss or sheen.

25. A method for making paint, said method comprising intimately mixing pulverized pitch and pulverized talc; and adding a sufficient quantity of a suitable solvent for the pitch to completely dissolve the pitch and render the paint freely flowable and brushable; the quantity of pitch being sufficient to form a binder and continuous cover for the talc, and a continuous pitch cover for the flowable paint and the structure to which it is applied; the quantity of talc being such as to give to the mass or paint a smooth flowability and smooth brushability and a gloss or sheen.

26. A method for making paint, said method comprising intimately mixing pulverized pitch and pulverized talc; and adding to the mixture a sufficient quantity of a suitable solvent for the pitch to quickly completely dissolve the pitch; the quantity of pitch being sufficient to form a binder and continuous cover for the talc and a continuous pitch cover for the flowable paint and the structure to which it is applied; the quantity of talc being sufficient to prevent the pitch from caking before adding the solvent, and such as to give to the paint a smooth flowability and such that the paint can have a gloss or sheen after polishing.

27. An easily flowing and brushable paint comprising intimately mixed powdered aggregate, mineral pitch and a solvent in which the pitch is completely dissolved; the quantity of solvent being such that the paint when cold is freely flowable and brushable and the pitch gives good surface protection.

28. An easily flowing, easily brushable paint comprising intimately mixed finely divided aggregate, mineral pitch and a solvent in which the pitch is completely dissolved; the pitch and aggregate being such as are free of affinity for or interaction with each other when powdered and dry; the quantity of solvent being such that the

paint is freely flowable and brushable; the proportion of pitch being such that the pitch causes the paint to give good surface protection.

29. An easily flowing, easily brushable paint comprising intimately mixed powdered aggregate and mineral pitch, and a solvent in which the pitch is completely dissolved the proportions of the pitch and aggregate being equivalent to 25 to 50 parts by volume of pulverized pitch to 50 to 75 parts of powdered aggregate; the pitch and aggregate being such as are free of affinity for or interaction with each other when powdered and dry; the quantity of solvent being such that the paint is freely flowable and easily brushable.

30. A method of the class described comprising intimately mixing finely pulverized dry mineral pitch and a finely divided dry aggregate; said pitch and aggregate being substantially free from interaction; and intimately mixing the mixture with enough of a suitable solvent to completely dissolve the pitch and form a freely flowable and brushable paint; said pitch being finely pulverized to render it conveniently quickly soluble in the solvent when making the paint; the proportion of pitch to aggregate being such that the pitch causes the paint to give good surface protection and said aggregate serves the function of mechanically separating the fine dry pitch particles before mixing with the solvent to prevent the compacting of the pitch particles together.

31. A method of the class described comprising intimately mixing about 50 parts by volume of pulverized dry mineral pitch and about 50 parts of a dry aggregate including shredded asbestos and hydrate of lime; said pitch and aggregate being when dry free from interreaction; maintaining said mixture free of moisture; and then intimately mixing the mixture with enough of a suitable solvent such as turpentine to quickly completely dissolve the pitch and form a freely flowable and brushable paint ready to be applied and hardened by evaporation of the solvent; said pitch being finely pulverized to render it conveniently quickly soluble in the solvent when making the paint; the proportion of pitch to aggregate being such that the pitch causes the paint to give good surface protection and said aggregate when dry serves the multiple function of retaining the pitch evenly distributed in the dry mixture before adding the solvent, mechanically separating the fine dry pitch particles to prevent the compacting of the pitch particles together before adding the solvent.

WILLIAM ZAISSER. 55